

# UNITED STATES PATENT OFFICE.

JOHN KEARNEY, OF KEENE, NEW HAMPSHIRE.

## BARREL-LINING.

SPECIFICATION forming part of Letters Patent No. 416,224, dated December 3, 1889.

Application filed March 7, 1889. Serial No. 302,324. (Specimens.)

*To all whom it may concern:*

Be it known that I, JOHN KEARNEY, a citizen of the United States, residing at Keene, in the county of Cheshire and State of New Hampshire, have invented certain new and useful Improvements in Compositions for Coating the Inside of Vessels Holding Oils, &c.; and I do declare the following to be a full, clear, and exact description of the invention, such as will enable others skilled in the art to which it appertains to make and use the same.

The object of my invention is to produce a cheap and efficient composition for coating the inside of all wooden or paper packages, cans, or vessels used for holding or transporting oils, paints, varnishes, benzine, spirits of turpentine, and all substances of an oily or pitchy nature, so as to render them proof against the penetration or action of said substances.

My composition consists of the following ingredients combined together in the proportions stated—viz., blood, seventy-five per cent.; dissolved glue, twenty-three per cent.; common potash, one per cent.; common salt, one per cent. The formula for combining or preparing said ingredients for use is as follows, viz: I first melt or dissolve a desired quantity of hard glue in the usual manner, by first adding the necessary amount of water, then boiling or steaming the same until it is dissolved into a liquid mass. I then add to the dissolved glue the proportionate quantity of potash and salt and stir well together while the glue is hot. The solution is then allowed to cool partially, so as to leave it simply lukewarm or at about 100° Fahrenheit. I then add the proportionate quantity of animal blood, as nearly fresh as can be obtained, and stir or agitate the mixture until it is thoroughly mixed. It then forms a compound of a dark-red color of the thickness or consistency of ordinary mixed paint, and is then ready for use. It is applied to the inside of open packages by means of a brush and to the interior of barrels or kegs by turning into the bung-hole a sufficient quantity and slushing the inside by rolling the vessel until the interior is thoroughly coated with the composition. The residue, if any, is then turned out.

The composition retains its liquid consistency while in bulk when cold, so that it can be applied while cold as well as when slightly warm. I find this quality quite a convenience for slushing barrels used for storing or transporting kerosene-oil, for the reason that when once prepared it is always ready for use.

After coating the vessel the compound dries as soon as ordinary paint and forms a smooth coating entirely impervious to the action of kerosene-oil and all greasy substances.

The potash acts as a solvent to the glue and blood and aids in forming a perfect solution of the ingredients. The salt I find to act in a similar manner, while both act as a preservative to the composition when stored in barrels, as well as after it is applied as a lining to the vessel. The salt and potash also render the composition less liable to crack when the vessel or package is exposed in dry places.

This composition can be produced much cheaper than any other preparation used for coating the inside of oil vessels or packages. The basis of the compound being animal blood, it can be obtained at slaughter-houses at a small cost as compared with glue.

I do not claim my composition is entirely impervious to the action of water; but it will resist the action of water much longer than preparations having a larger proportion of glue.

Having fully described my invention, I claim—

The process of rendering wooden or paper vessels or packages proof against the action or penetration of oils, paints, varnishes, benzine, spirits of turpentine, pitch, and kindred substances, which consists in coating the inside thereof with a composition consisting of a solution of blood, dissolved glue, carbonate of potassium, and chloride of sodium when prepared in the manner and in the proportions above set forth.

In testimony whereof I affix my signature in presence of two witnesses.

JOHN KEARNEY.

Witnesses:

HIRAM BLAKE,  
E. M. FLINT.